

[72] Inventor **Arthur W. Sperling**  
Amityville, N.Y.  
[21] Appl. No. **734,194**  
[22] Filed **June 4, 1968**  
[45] Patented **Jan. 4, 1972**  
[73] Assignee **Hogan Faximile Corporation**  
Los Angeles, Calif.

[54] **NONBLOCKING ELECTROLYTIC RECORDING MEDIUM**  
9 Claims, No Drawings

[52] U.S. Cl..... **117/201,**  
117/161 ZA, 204/2, 117/155 UA  
[51] Int. Cl..... **B44d 1/02**  
[50] Field of Search..... **117/201,**  
155 V, 161 ZA; 204/2; 346/74

[56] **References Cited**  
UNITED STATES PATENTS  
3,335,221 8/1967 Barnes et al. .... 346/74 X  
3,123,542 3/1964 Mandel et al. .... 204/2  
3,342,704 9/1967 Gradsten et al. .... 204/2  
3,344,043 9/1967 Lieblich et al. .... 204/2  
3,459,593 8/1969 Cole ..... 117/155 V X

*Primary Examiner—Alfred L. Leavitt*  
*Assistant Examiner—Caleb Weston*  
*Attorneys—Samuel Lindenberge and Arthur Freilich*

**ABSTRACT:** A nonblocking electrolytic recording medium is disclosed. The medium includes a base sheet of absorbent paper impregnated at a level of at least 40 percent by weight of moisture with an electrolytically conducting marking solution. The solution contains an aqueous dispersible liquid silicone, preferably 0.005 to 2.0 grams per 100 milliliters of a polymethyl-siloxane having a viscosity at 25° C. between about 10 to about 100 centistokes.

## NONBLOCKING ELECTROLYTIC RECORDING MEDIUM

## BACKGROUND OF THE INVENTION

## 1. Field of the Invention

This invention relates to electrosensitive recording media and more particularly to an improved, nonblocking recording medium.

## 2. Description of the Prior Art

An electrolytic recording medium of the type utilized in facsimile recorders is prepared by impregnating an absorbent base sheet with an electrolytically conducting solution containing a marking compound. In the recorder that is now in general use, marking is effected by disposing the impregnated paper between a stationary blade anode electrode and a cooperating rotating helical cathode. When a voltage is applied between the electrodes, current flows through the paper at the moving intersection of the electrodes. Metal ions supplied by electrolytic dissolution of the anode react with the marking compound to form a colored mark on the surface of the paper wherever the anode contacts the paper adjacent the oppositely disposed cathode.

Large volumes of this paper are consumed in the facsimile-recording machines utilized by the wire services. Continuous production of exact copy is imperative and, therefore, the paper must satisfy several very important specifications. The paper must have the ability to produce marks having a density which is a function, preferably linear, of the current passed through the paper. The marking compound must produce color tones varying uniformly through a range from white at zero current flow through grays for intermediate magnitudes of current to black for the highest or maximum current magnitudes. There should be a minimum of bleeding or fringing of the mark so as to maintain a sharply detailed and defined recorded image.

The wet paper is stored at high humidity in special containers for extended periods prior to use in a recorder and must remain stable without chemical decomposition or loss of ingredients which would cause discoloration of the paper before use or background discoloration after being recorded. It is also desirable to employ a paper that is insensitive to light even after exposure to ultraviolet light as in Ozalid duplicating machines.

In many of the present electrolytic recording papers, a polyhydroxyphenolic such as catechol has a tendency to diffuse or transfer out of the paper and discolor adjacent sheets of paper and other surfaces such as the recorder cabinet and walls of the room containing the recorder.

Moreover, bearing in mind that wire service facsimile machines are in almost continuous use, it is not uncommon to encounter a condition in which current flow through the electrodes is hindered or blocked by the accumulation of fibers or precipitated salts on the helical blade. The impedance to current flow phenomena at these points has been commonly referred to as "blocking." When current is blocked, no mark can be formed until the materials are dislodged from that portion of the blade. Moreover, the salting out or precipitation of the materials present in the impregnant may result in a discoloration of the background of the sheet.

## OBJECTS AND SUMMARY OF THE INVENTION

It is therefore an object of the invention to provide an improved electrosensitive graphic recording media.

Another object of the invention is the provision of an improved nonblocking electrolytic recording medium.

Another object of the invention is to provide a nonblocking electrosensitive recording medium which contains a nontransferring marking ingredient and which is not susceptible to background discoloration before and after recording.

Other objects and many attendant advantages of the invention will become apparent to those skilled in the art as the description proceeds.

In accordance with the invention, it has been discovered that a nonblocking stable, electrosensitive recording medium is prepared by impregnating a porous support with an aqueous solution containing a mark-forming compound, an electrolyte and a water-dispersible, organic silicone polymer. The electrosensitive recording medium of the invention does not result in any blocking even after being run for considerable periods through the same facsimile-recording apparatus. The paper is stable to light and does not discolor either before or after recording and the marks that are formed are clear and distinct.

The invention will become better understood by reference to the following detailed description.

## BRIEF DESCRIPTION OF THE PREFERRED EMBODIMENTS

In accordance with the present invention, the water-dispersible, organic silicone polymer is preferably a linear organic polysiloxane of the formula:



where R is preferably lower alkyl such as methyl or ethyl, but can also be aryl such as phenyl or hydroxy, amino, lower alkenyl or lower alkoxy, and n is an integer between 0 and 2,000. The polymer is an oily liquid exhibiting a viscosity which can be varied within wide limits, but preferably is from about 5 to 500 centistokes (cs.) at 25° C. and most suitably from 10 to 100 cs. Polydimethylsiloxanes in amounts from about 0.005 to 2.0 grams per 100 milliliters of water are found to disperse readily to form electrolytic recording media.

The marking agents are typically polyhydroxyaromatic compounds in which at least two of the phenolic hydroxyl groups are ortho to each other. The aryl ring nucleus may be substituted with various other substituents to vary certain properties such as vapor pressure and stability. Such compounds may be selected from those of the following general formula:



where R<sup>a</sup>, R<sup>b</sup> and R<sup>c</sup> are lower alkyl, amino, lower alkoxy, aryloxy, carboxy, sulfoxy, hydroxy, lower alkanoyl, lower alkenoyl, halo or hydrogen. R<sup>d</sup> is R<sup>a</sup> or R<sup>c</sup>X where X is carboxy or sulfoxy, and R<sup>e</sup> is -(CR<sup>a</sup>R<sup>b</sup>)<sub>n</sub> or -NH-(CR<sup>a</sup>R<sup>b</sup>)<sub>n</sub> where n is an integer from 1 to 10, and R<sup>f</sup> and R<sup>g</sup> are hydrogen, hydroxyl, amino or lower alkyl. The -(CR<sup>a</sup>R<sup>b</sup>)<sub>n</sub> group may be unsaturated. Condensed nuclear aromatic compounds may also be used as marking compounds. For example, hydroxynaphthalene compounds such as hydroxynaphthoic acid is a suitable marking compound. Other examples of marking compounds are gallic acid, catechol, pyrogallol, gentisic acid, chromotropic acid, protocatechuic acid, caffeoic acid and a dihydroxyphenyl alcanoic acid such as 3, 4-dihydroxyphenylacetic acid (DHPAA).

DHPAA and analogous compounds are advantageous in that the capability of transferring from the paper is substantially reduced. However, at concentrations desired for optimum electrolytic marking, DHPAA is poorly soluble in the media and tends to crystallize out further aggravating the blocking phenomena previously discussed. The water-dispersible silicone-containing formulations of the invention are particularly effective in eliminating the blocking of electrolytic

recording media containing poorly soluble compounds such as DHPAA. This class of compounds is represented by compounds of the general formula:



where  $\text{R}^a$ ,  $\text{R}^b$ , and  $\text{R}^c$  may be lower alkyl, amino, lower alkoxy, hydroxy, lower alkanoyl, halo, or hydrogen.  $\text{R}^d$  may be an alkylene or amino-alkylene moiety of the formula  $-(\text{CR}^e\text{R}^f)-$  or  $-\text{NH}(\text{CR}^e\text{R}^f)_n-$  where  $n$  is an integer from 1 to 10, and  $\text{R}^e$  or  $\text{R}^f$  may be H, lower alkyl, amino, hydroxy or other suitable substituents. X is  $-\text{COOH}$  or  $-\text{SO}_3\text{H}$ . Examples of other suitable marking compounds within this class are 3, 4-dihydroxybetaphenylpropionic acid (DHPPA) and 3, 4-dihydroxyaniline-N-methyl-sulfonic acid (DHAMSA).

The recording medium generally comprises an absorbant, inert, porous and preferably white support such as a sheet of paper having a high wet strength which is impregnated with an aqueous solution of an electrolytic recording impregnant. The impregnant contains the marking compound, an electrolyte and usually, also a stabilizer, an acidifier and one or more antifringing agents.

Recording paper is prepared by passing the porous sheet through a bath of impregnant. Approximately 2.5 to 3.0 cc. of the solution is required per square foot of paper in a typical case. The solution is permitted to distribute itself throughout the paper. Excess impregnant is removed by passing the paper through pressure rolls until at least about 40 percent moisture by weight remains. In order to retard evaporation, the recording paper is generally stored in sealed containers until needed for recording.

A typical formulation with which recording paper may be impregnated is now given by way of illustration.

#### EXAMPLE 1

About 0.4 grams of Dow Corning 200, a polydimethylsiloxane having a viscosity of 100 centistokes at 25° C. was dispersed into 100 ml. of water. The following ingredients were then added with stirring.

|                      |           |
|----------------------|-----------|
| NaCl                 | 14.6 g.   |
| NaClO <sub>3</sub>   | 4.0 g.    |
| DHPAA                | 2.75 g.   |
| Thiourea             | 0.5 g.    |
| Oxalic acid          | 0.0875 g. |
| Monosodium Phosphate | 0.1 g.    |

The solution of example 1 was filtered and it was observed that the silicone oil did not separate out. The solution was then permitted to stand overnight and again, no separation of the silicone oil was evidenced.

A control impregnant was prepared having the identical composition except that the silicone was not present.

A series of hand sheets were impregnated with the solution of example 1 and the control impregnant. The papers were hung side by side in a window to expose them to sunlight. The hand sheet of example 1 was found to be less affected by ultraviolet light.

The quantity of DHPAA may be varied up to the solubility limit thereof which is approximately 40 grams per 100 cc. of solution. The sodium chloride electrolyte may be replaced with another group I or group II metal chloride, bromide or nitrate. The chlorides and bromides are preferred since papers made with nitrates exhibit substantially more discoloration when exposed to ultraviolet light. Sodium chloride may be present in quantities varying from zero to its solubility limit at about 30 grams per 100 cc. of solution and the exact quantity depends upon the degree of electrical conductivity desired.

Thiourea functions as a stabilizer in the composition of the invention and may be replaced by other compounds such as lower alkyl derivatives of thiourea or dithiobiuret. The thiourea may be varied from about 6.1 grams which is the limit for stability to about 10 grams per 100 cc. of solution which is the approximate solubility limit.

The pH of the paper is preferably maintained in the range of from about 1.0 to 3.5 by addition of an acid such as oxalic and a buffer such as monosodium phosphate. At a pH value about 10 3.5, the mark is apt to change color and at a pH of less than 1, the mark is generally of lighter density than acceptable.

The monosodium phosphate also provides an antifringing function. It may be present in amounts ranging up to about 0.5 grams above which it tends to decrease the density of the mark. The sodium chloride produces additional marking density by oxidizing the metal ions to a higher valency state and is also believed to increase the density of the mark by polymerization, especially when the recording is heated after the mark has formed. DHPPA gives marks of excellent density when used in conjunction with oxidizing agents such as sodium chlorate.

During the recording process, a recorder is employed in which an electric current is passed through the recording paper while it is sandwiched between a rotating helical cathode and a stationary bar anode which are in contact with opposite surfaces of the paper. The anode may be composed of iron, stainless steel, silver or some other eroding metal capable of electrolytic dissolution to form ions which react with the marking compound to form one or more colored complex compounds which constitute the recorded colored marks. The recorded paper may then be dried in air or by some heating device to permanently fix the recorded marks. The formulations of example 1 and the control were impregnated into wet strength paper and the moisture content adjusted to 40 percent. A new stainless steel printer blade was inserted into a recorder and the helix thoroughly cleaned. Comparison runs of 108 inches of 8.5 inch wide paper were run through the recorder. Copy was run white at no current, then black at maximum current density. Upon the completion of each run, the helix was examined closely for pickup. With the control paper, after approximately 25 feet of no current and then maximum marking current, accumulation of material on the helix occurred with blocking of the current and blank spots on the record. With the paper impregnated with the solution of example 1, the recorder ran smoothly throughout the complete run. A thin layer of nonoily black material was observed to have gathered on the blade. This material was easily removable. The material collected only on the side of the blade which was in contact with the helix through the paper. Production run rolls of paper were prepared and recorded in a standard wire service recorder under in-service conditions. No blocking effect was observed after several 400-foot rolls of paper had been run between the helix and the blade.

It is understood that only preferred embodiments of the invention have been disclosed and that numerous substitutions, alterations and modifications are all permissible without departing from the spirit and scope of the invention as defined in the following claims.

What is claimed is:

1. An electrolytic recording medium comprising: an impregnated sheet containing; an aqueous electrolytically conducting solution at a level of at least 40 percent by weight of moisture; said solution including a polyhydroxy-aromatic marking compound; and an even dispersion of an aqueous dispersible, liquid, organic polysiloxane polymer having a viscosity at 25° C. of from 5 to 500 cs. and being present in said solution in an amount of 0.005 to 2.0 grams per 100 ml. of water.
2. A medium according to claim 1 in which the polysiloxane has a viscosity at 25° C. of from about 10 to 100 centistokes.
3. A medium according to claim 2 in which the polysiloxane is selected from polymers of the formula:



where R is lower alkyl, aryl, hydroxy, amino, lower alkenyl or lower alkoxy and n is an integer from 0 to 2,000.

4. A medium according to claim 3 in which R is methyl.

5. A medium according to claim 1 in which the marking compound is a polyhydroxy-aromatic compound containing at least two phenolic hydroxyl groups which are ortho to each other.

6. A medium according to claim 5 in which the marking compound is selected from those of the formula:



5

where R<sup>a</sup>, R<sup>b</sup> and R<sup>c</sup> are lower alkyl, amino, lower alkoxy, lower alkanoyl, halo or hydrogen; and

R<sup>d</sup> is R<sup>a</sup> or R<sup>a</sup>X where R<sup>a</sup> is lower alkylene or aminoalkylene and X is carboxyl or sulfoxyl.

7. A medium according to claim 6 in which the marking compound is a dihydroxyphenyl alkanoic acid.

8. A medium according to claim 7 in which the marking compound is dihydroxy phenylacetic acid.

9. An electrolytic recording medium comprising:  
a sheet of paper impregnated with an aqueous solution at a level of at least 40 percent by weight of moisture; said solution containing on a basis of 100 ml. of water; 0.005 to 2.0 grams of a liquid polymethylsiloxane; having a viscosity of from 10 to 100 cs.

10

15 up to 30 grams of a group I or group II metal chloride, bromide or nitrate; 0.1 to 5 grams of a thiourea compound; up to 0.5 grams of monosodium phosphate; and up to 40 grams of dihydroxy phenylacetic acid.

20

\* \* \* \* \*

25

30

35

40

45

50

55

60

65

70

75